

## UNITED STATES PATENT OFFICE

2,228,310

## METHOD FOR PRODUCING BERYLLIUM ALLOYS

Herbert Gruber, Werner Hessenbruch, and Wilhelm Rohn, Hanau, Germany, assignors to Heraeus-Vacuumschmelze, A. G., Hanau-on-the-Main, Germany

No Drawing. Application March 13, 1939, Serial No. 261,649. In Germany March 25, 1938

8 Claims. (Cl. 75—153)

This invention relates to a method for producing beryllium alloys, more particularly alloys of beryllium with heavy metals, especially with copper.

5 It is known that beryllium alloys of this type can be produced by reducing beryllium oxide with carbon in the presence of a molten bath of the metal with which the beryllium is to be alloyed. For example, the bath may be composed of 10 copper, or a metal of the iron group (iron, nickel, cobalt), or a metal of the chromium group (chromium, molybdenum, tungsten, uranium), or a molten bath containing a mixture or an alloy of several of these metals may be used.

15 One of the most important beryllium-heavy metal alloys is the copper-beryllium type, and by following the above general procedure, using copper for the molten bath, an alloy may be produced having a beryllium content anywhere up to 20 about 3.5-4%. However, difficulties are encountered when attempts are made to operate in a manner to produce a beryllium-copper alloy having a higher beryllium content. For economic reasons it is desirable to be able to produce a 25 higher-percentage beryllium master alloy, which could then be employed for the production of beryllium-copper alloys having lower beryllium content, for instance, from about 1.5 to about 2.5%, by diluting with more copper.

30 It has been known that beryllium-copper alloys of the type having a percentage of beryllium up to about 3.5 to 4%, may be produced by the thermic reduction method briefly described above, the alloys being practically carbon-free, especially 35 if after the reduction is ended the excess carbon is caused to rise by twirling or spinning the metal bath, in the general manner in which kish graphite is removed.

Certain of the difficulties which are encountered when attempting to produce beryllium-copper alloys having a beryllium percentage above about 4%, are not encountered when operating with a molten bath of one or more of the metals nickel, cobalt and iron. With these metals 45 of the iron group, especially with nickel or cobalt, an alloy containing from about 12-15% beryllium, balance nickel or cobalt, may effectively be produced. The operating costs involved in this procedure are substantially the same as those for the 50 production of a 2-4% beryllium-copper alloy, and therefore the production costs of a given weight of beryllium content in the beryllium-nickel alloys are less than in the case of the beryllium-copper alloys.

55 However, it has been found that in producing a

beryllium-nickel alloy, substantial quantities of carbon remain dissolved, this difficulty being especially noticeable when the reaction takes place in air. While the quantity of dissolved carbon can be reduced by remelting the alloy in the presence of further beryllium oxide, and preferably under reduced pressure, this procedure is disadvantageous since a considerable loss of beryllium results due to the fact that beryllium and beryllium carbide evaporate. In consequence, removing the dissolved carbon in this way results in a drop in the beryllium content from the initial quantity of about 12-15% down to about 5-7%.

With the foregoing difficulties in mind, the present invention contemplates production of a beryllium-heavy metal alloy, especially a beryllium-copper alloy, by first reducing beryllium oxide with carbon in the presence of a molten bath of nickel, cobalt or iron, to produce a beryllium-nickel alloy containing, for example, from 12-15% beryllium. In producing a beryllium-copper alloy this beryllium-nickel alloy is then diluted with a substantial quantity of copper, which has the effect of precipitating the dissolved carbon.

The amount of dilution necessary in most instances to accomplish the precipitation of the carbon is from about 35-40%, although for most purposes it is found desirable that the copper should heavily predominate in the final alloy, the copper being preferably in excess of 75%.

The reduction of the beryllium oxide in the presence of the molten bath may take place in air, or in the vacuum chamber, or in the hydrogen atmosphere. If desired, lime, or calcium carbide or other similar fluxes may be used.

It should also be noted that it is not necessary to employ pure beryllium oxide in carrying out the reaction. The beryllium oxide may be present in the form of ore, in which event other oxides may be present. The beryllium oxide may be mixed with the carbon in the form of graphite or in the form of a carbide, especially beryllium carbide, and this mixture then introduced into the molten bath.

The amount of copper added to dilute the alloy first produced (for instance the beryllium-nickel alloy) may be such as to produce a beryllium content from about 3-10%. In most instances, however, it is preferable that the dilution should be sufficient to result in a copper content well over 75%.

As an example, a beryllium-nickel alloy may first be produced containing 15% beryllium, and

this alloy then diluted with about seven times its weight of copper, thereby resulting in an alloy containing about 87.5% copper, about 2% beryllium, and the balance nickel. An alloy having the beryllium and nickel percentages of about the order just indicated, is found to have physical properties essentially equivalent to a comparable alloy of beryllium and copper alone, especially with respect to high mechanical hardness, elasticity, and wear and fatigue resistance. The alloy containing nickel (in addition to the beryllium and copper) can be heat treated by precipitation hardening in much the same way as pure beryllium-copper alloys, i. e. by quenching from temperatures between about 600° and 800° C. and then annealing at temperatures between about 250° and 400° C.

As another example of the application of the invention, reference is made to the use of a molten cobalt bath, for the purpose of producing first a beryllium-cobalt alloy and then diluting this alloy with copper, the operation being carried out, for instance, to result in a beryllium content of about 4% and a cobalt content of about 2.6%, copper representing the balance. Alloys of this general class are outstanding for certain purposes because of possessing particularly high hardness, coupled with good electrical conductivity, making them especially suitable for welding electrodes, switches, contact parts and the like.

It will be apparent also that various mixtures of nickel, cobalt and iron may be used, depending upon the purposes for which the alloy is being prepared. Similarly, the extent of dilution with copper will vary in accordance with the properties desired.

In instances where it is desirable to have silicon present in the alloy in addition to the beryllium, the invention contemplates addition of silicon either to the molten bath initially or simultaneously with the beryllium oxide. Since silicon reduces the solubility of carbon in metals of the iron group, when using a molten nickel, cobalt or iron bath, very little if any carbon remains. The addition of silicon is also advantageous because it reduces the melting point of the master alloys produced in view of which such master alloys will dissolve more rapidly and easily in a molten bath of copper which may be used for dilution.

As an example of the use of silicon, reference may be made to the production of an alloy suitable for welding electrodes, in which a silicon content in the neighborhood of .5% is desirable. Thus, when producing an alloy for welding electrodes having in the neighborhood of .5% beryllium, silicon may be added to the molten bath in an amount equivalent to the quantity of beryllium which is to be reduced therein.

When operating in the manner according to which silicon is added to the molten bath, since the carbon content is thereby kept at a very low value, the alloys produced may, if desired, be diluted with other metals such, for example, as nickel or cobalt or iron, instead of with copper, and thereby nickel, or cobalt, or iron base alloys may be obtained, which are very low in carbon.

In all examples according to the invention, it is possible to produce an initial alloy having high beryllium content which initial alloy may subsequently be diluted, the dissolved carbon being reduced either at the time of reduction (by the addition of silicon) or at the time of dilution (by dilution with copper).

We claim:

1. The method of producing a substantially carbon-free alloy containing beryllium and copper and in which the copper heavily predominates over the other ingredients, which method includes bringing into reaction beryllium oxide and carbon in the presence of a molten bath of a metal chosen from the group consisting of nickel, cobalt and iron to produce an alloy of beryllium and said metal and in which carbon is also present, thereafter diluting the alloy with copper in an amount providing a copper content of at least 35%, to precipitate the carbon remaining in the alloy from said reaction. 10

2. The method of producing a substantially carbon-free alloy containing beryllium and copper and in which the copper heavily predominates over the other ingredients, which method includes bringing into reaction beryllium oxide and carbon in the presence of a molten bath of a metal chosen from the group consisting of nickel, cobalt and iron to produce an alloy of beryllium and said metal in which the beryllium constitutes from about 12-15%, and thereafter diluting the alloy with copper in an amount between that lower limit which will provide an alloy containing at least about 35% copper and that upper limit which will provide an alloy containing at least about .3% beryllium. 20

3. The method of producing a substantially carbon-free alloy containing beryllium and copper and in which the copper heavily predominates over the other ingredients, which method includes bringing into reaction beryllium oxide and carbon in the presence of a molten bath of a metal chosen from the group consisting of nickel, cobalt and iron to produce an alloy of beryllium and said metal in which the content of the metal of said group heavily predominates over the beryllium but in which the beryllium content 35 constitutes several times the percentage ultimately desired, and thereafter diluting the alloy with copper in an amount such that the copper constitutes at least 75% of the alloy. 40

4. The method of producing a substantially carbon-free alloy containing beryllium and copper and in which the copper heavily predominates over the other ingredients, which method includes bringing into reaction beryllium oxide and carbon in the presence of a molten bath of a metal chosen from the group consisting of nickel, cobalt and iron to produce an alloy of beryllium and said metal in which the beryllium constitutes in the neighborhood of 12-15% of the alloy, and thereafter diluting the alloy with copper in an amount sufficient to reduce the beryllium content to a percentage of the order of 2%. 50

5. The method of producing a substantially carbon-free alloy containing beryllium and copper and in which the copper heavily predominates over the other ingredients, which method includes bringing into reaction beryllium oxide and carbon in the presence of a molten bath of cobalt to produce a beryllium-cobalt alloy in which the cobalt heavily predominates and in which a substantial amount of carbon is also present, and thereafter diluting the alloy with copper to precipitate the carbon and to reduce the beryllium content to a percentage of the order of 4%. 60

6. The method of producing a substantially carbon-free alloy containing beryllium and copper and in which the copper heavily predominates over the other ingredients, which method includes bringing into reaction beryllium oxide 70

and carbon in the presence of a molten bath of a metal chosen from the group consisting of nickel, cobalt and iron and also in the presence of silicon to produce an alloy of beryllium, silicon and the metal of said group in which the beryllium constitutes from about 12-15%, and thereafter diluting the alloy with copper in an amount between that lower limit which will provide an alloy containing at least about 35% copper and that upper limit which will provide an alloy containing at least about .3% beryllium.

7. The method of producing a substantially carbon-free alloy containing beryllium and copper and in which the copper heavily predominates over the other ingredients and in which the beryllium constitutes from about .3% to about 10% of the alloy, which method includes bringing into reaction beryllium oxide and carbon in the presence of a molten bath of a metal chosen from the group consisting of nickel, cobalt and iron and also in the presence of a quantity of silicon approximately equal to the quantity of beryllium to be reduced in the metal of said group to produce an alloy of beryllium, silicon and the metal of said group in which the beryllium constitutes from about 12-15%, and thereafter di-

luting the alloy with copper in an amount between that lower limit which will provide an alloy containing at least about 35% copper and that upper limit which will provide an alloy containing at least about .3% beryllium.

8. The method of producing a substantially carbon-free alloy of beryllium with a heavy metal in which the heavy metal content heavily predominates over the other ingredients, which method includes bringing into reaction beryllium oxide and carbon in the presence of a molten bath of a metal chosen from the group consisting of nickel, cobalt and iron and also in the presence of silicon to produce an alloy of beryllium, silicon and the metal of said group very low in carbon in which the beryllium constitutes from about 12-15%, and thereafter diluting the alloy with a heavy metal in an amount between that lower limit which will provide an alloy containing at least about 35% of said heavy metal and that upper limit which will provide an alloy containing at least about .3% beryllium.

WILHELM ROHN.  
HERBERT GRUBER. 25  
WERNER HESSENBRUCH.